

## UNITED STATES PATENT OFFICE

2,246,541

## SAFETY PAPER

John Q. Sherman and Wilbur A. Yackley, Dayton,

Ohio; said Yackley assignor to said Sherman;

Katherine M. Sherman, William C. Sherman,

and Wellmore B. Turner, executors of John Q.

Sherman, deceased

No Drawing. Application January 7, 1937,  
Serial No. 119,524

8 Claims. (Cl. 91—67.95)

This invention pertains to paper manufacture and comprises a safety paper suitable for checks, vouchers, money orders, valuable records, agreements and legal papers which it is desired to protect against change and more particularly to a paper which is adapted to visually indicate any attempt to tamper therewith and efforts to change or add to a written record.

Safety paper is now commonly employed whereon attempted erasures become plainly visible but do not deter attempts of a skilled penman to change the written record by adding to or reforming existing letters or words to raise the amount of a check or voucher or change a signature or the import of written matter without necessity of making erasures.

The present paper has the conventional surface and appearance of ordinary writing or printing paper and bears no visible indication which will forewarn a forger or others of its peculiar character. However, the paper is so treated, either during manufacture or by surface application thereafter, that when written upon with ordinary commercial inks such as are generally available, the ink lines will spread or "feather out" as upon blotting paper. However, the paper is susceptible of being written upon in the ordinary manner with specially prepared ink which produces thereon a written record having the natural and normal appearance made by conventional inks.

The purpose of the invention is to provide a protective paper which will readily indicate any attempt to change the record thereon or add thereto, even though no erasure be made, and thereby serve as a deterrent to dishonesty.

An important object of the invention is to provide a safety paper which may be economically manufactured and which will possess a normal conventional appearance, the special character of which is concealed.

A further object of the invention is to provide a protective paper which will be incapable of receiving legible records when written in ordinary commercial ink such as are generally available, but which will legibly receive written records when made with a specially prepared ink.

A further object of the invention is to provide a suitable ink for use upon the specially prepared paper herein described.

With the above primary and other incidental objects in view as will appear in the specification, the invention consists of the materials and the combination thereof, and the process of manufacture and mode of operation herein described and set forth in the claims.

The safety paper herein described, is produced by treating ordinary paper with conditioning mixture of a pigment such as titanium oxide, an alcohol such as glycerol, water and a silicate of which sodium silicate is a suitable material. With no intent to unduly limit the scope or application of the invention, but merely for illustrative purpose, the following formula of ingredients and proportions thereof has been found quite effective:

|                  | Per cent |
|------------------|----------|
| Titanium dioxide | 14.15    |
| Glycerol         | 4.69     |
| Water            | 35.46    |
| Sodium silicate  | 45.75    |

In preparing the mixture the pigment is ground in the water and alcohol and the silicate is subsequently added and the grinding operation continued until the pigment is thoroughly dispersed throughout the media. If the paper is to be tinted, a dye material such as crocein scarlet concentrate is added to the mixture in sufficient quantity to impart the desired shade of color.

The media thus prepared may be incorporated in the paper pulp material during its manufacture or it may be applied to the paper while being formed on the Fourdrinier machine or as it leaves such apparatus. Preformed paper may be treated by dipping it in the treatment media, or by brushing it onto the surface of the paper. In some instances it may be desirable to treat only isolated areas of the paper stock upon which written inserts are to be made, in which case the material is necessarily applied to previously manufactured paper, preferably by an imprinting operation whereby the media may be applied only throughout well defined spaced areas.

Upon application of ordinary commercial writing inks to the treated paper the ink lines will spread or "feather out" into a fuzzy blur similar to its action on blotting paper. It is found that some inks in general use will fade and lose their colors quite rapidly when applied to such treated surface. It is quite impossible to write legibly upon such specially treated paper with ordinary inks. The treated paper being of ordinary appearance does not indicate in advance its peculiar nature and hence affords no forewarning.

In order to produce legible records on the treated paper a special writing fluid is employed consisting of a fast dye of which victoria blue base concentrate is an example, combined with a pigment such as iron blue, an alcohol of which a

synthetic gum of polyvinyl acetate type is deemed suitable.

A typical formula stated for illustrative purpose, but not as a limitation comprises:

|                | Per cent |
|----------------|----------|
| Dye or pigment | 7.52     |
| Alcohol        | 30.07    |
| Gum            | 62.41    |

In preparing this writing fluid the gum and pigment are ground in the alcohol until thoroughly dispersed and of uniform character. This writing fluid does not "run" or "feather out" as does ordinary commercial ink when applied to the treated paper surface but produces a clear legible line which is of fast color which takes on a permanent darker hue when subjected to light.

Inasmuch as safety paper is extensively used for printing purposes, in the production of checks, vouchers and the like, it has been found desirable to produce a complementary printing ink for use thereon.

Such printing ink comprises a fast type such as victoria blue base concentrate, or a pigment of which iron blue is an example, combined with a lithographic varnish, a drier material such as cobalt or manganese oxide and a suitable wax of which bees wax is found satisfactory and a plate oil.

Typical formulae submitted for illustrative purposes comprise:

*Formula A*

|                      | Per cent |
|----------------------|----------|
| Lithographic varnish | 44       |
| Plate drier          | 3        |
| Pigment or dye       | 52       |
| Wax                  | 1        |

*Formula B*

|                |    |
|----------------|----|
| Plate oil      | 33 |
| Pigment or dye | 43 |
| Drier          | 24 |

The herein described treatment of the paper renders it more absorptive than ordinary papers or increases the capillary attraction effect thereof whereby ordinary writing fluid which is slow drying will be rapidly absorbed and will be drawn by the increased capillary attraction into a more widely spread area. The prescribed ink for writing on such prepared paper having a gum base is more viscous and more rapid drying and hence resists the capillary attraction and does not spread or "feather out" as does ordinary ink.

In the formula which is here stated merely for illustrative purpose, it being understood that other materials of analogous character may be substituted therefor, the titanium affords the absorbent characteristic while the sodium silicate is used as a binder, and the glycerol as a plasticiser to prevent excessive hardening and make the coating pliable. The water is merely the vehicle to render the mixture sufficiently fluid for application. The alcohol which renders the ink initially more fluid rapidly evaporates after application to the paper leaving the remaining deposit of gum and pigment even more viscous and hence with less tendency to spread. The gum being of a quick drying character the ink sets rapidly, and hence may be successfully used upon absorbent surfaces such as afforded by the paper treatment material.

From the above description it will be apparent that there is thus afforded paper treatment material and a complementary ink and method of

operation of the character described possessing the particular features of advantage before enumerated as desirable, but which obviously is susceptible of modification in its form, proportions, detail construction and arrangement of parts without departing from the principle involved or sacrificing any of its advantages.

While in order to comply with the statute, the invention has been described in language more or less specific as to structural features, it is to be understood that the invention is not limited to the specific features shown, but that the means and construction herein disclosed comprise the preferred form of several modes of putting the invention into effect, and the invention is, therefore, claimed in any of its forms or modifications within the legitimate and valid scope of the appended claims.

Having thus described our invention, we claim:

1. A protective record including the combination of a record material simulating the appearance of ordinary record material to be written upon, and having a porous, absorptive surface, and a non-penetrating ink for use therewith sufficiently viscous to resist capillary attraction of the absorbent record material and produce lines and characters in simulation of those produced by ordinary ink on ordinary writing material.

2. The herein described method of making records which includes treating a writing material to increase the normal capillarity thereof while maintaining the normal appearance of the writing material, and writing on the material with an ink sufficiently volatile to resist the effect of the increased capillarity of the writing material and produce sharply defined lines and characters in simulation of characters producible with ordinary ink on the writing material prior to such treatment thereof.

3. A protective record including a writing material simulating ordinary writing material in appearance and having a degree of capillarity in excess of that of ordinary writing material, and an inscription thereon in a complementary ink resistant to the excess capillarity of the writing material and which produces sharply defined lines and characters when applied thereto in simulation of those produced on ordinary writing material by ordinary ink.

4. In a protective record, the combination with a record material simulating ordinary writing material in appearance and having a degree of capillarity in excess of that of ordinary record material and such as to effect rapid spreading of ordinary ink, of a complementary ink sufficiently non-flowing upon exposure to air as to resist the capillarity of the record material and produce sharply defined lines and characters when applied thereto in simulation of those produced on ordinary writing material by ordinary ink.

5. A writing material treated with an absorbent, a plasticizer and a binder material to increase the capillarity thereof over and above the normal capillarity of ordinary writing material while simulating the appearance of ordinary writing material, whereby the writing material is rendered incapable of receiving legible inscriptions written in other than writing fluid sufficiently non-flowing upon application to the treated material as to resist the increased capillarity of the treated writing material and produce lines and characters in simulation of those produced by ordinary ink on ordinary writing material.

6. A writing material treated with a mixture

of titanium dioxide, glycerol and sodium silicate to increase the capillarity thereof over and above that of ordinary writing material, whereby the writing material is rendered incapable of receiving legible inscriptions written in other than writing fluid sufficiently non-flowing upon application to the writing material as to resist the increased capillarity of the treated writing material and thereby produce sharp lines and characters when applied thereto in simulation of lines and characters produced by ordinary ink on ordinary writing material.

7. In a protective record, the combination with a record material simulating ordinary writing material in appearance and having a degree of capillarity in excess of that of ordinary writing material and rendering it incapable of receiving legible inscriptions written in other than writing fluid sufficiently non-flowing upon application to the record material as to resist the capillarity thereof to produce lines and characters in simu-

lation of those produced by ordinary ink on ordinary writing material, of an ink for use therewith including approximately 7% pigment, 62% gum and 30% volatile solvent.

8. A writing material treated with a mixture of approximately 14% titanium dioxide, 4% glycerol, 45% sodium silicate and 35% water to increase the capillarity thereof over and above that of ordinary writing material, whereby the writing material is rendered incapable of receiving legible inscriptions written in other than writing fluid sufficiently non-flowing upon application to the writing material as to resist the increased capillarity of the treated writing material and thereby produce sharp lines and characters when applied thereto in simulation of those produced by ordinary ink on ordinary writing material.

JOHN Q. SHERMAN.  
WILBUR A. YACKLEY.